

March 30, 1937.

F. GETTELMAN

2,075,518

ART OF SURFACING ONE METAL WITH ANOTHER

Filed Oct. 4, 1934

*Fig. 1.*



*Fig. 2.*



INVENTOR

Frederick Gettelman

BY  
Wheeler, Wheeler & Wheeler

ATTORNEYS

## UNITED STATES PATENT OFFICE

2,075,518

ART OF SURFACING ONE METAL WITH  
ANOTHER

Fredrick Gettelman, Milwaukee, Wis.

Application October 4, 1934, Serial No. 746,831

3 Claims. (CL 91—70.1)

This invention relates to improvements in the art of surfacing one metal with another.

It is the primary object of the invention to provide means for producing mechanically the 5 equivalent of a metallic plating operation. While the invention is applicable to metal sheets, it is of particular importance in the surfacing of the interiors of metal containers to produce a smooth surface metallic ply.

10 At present composite sheets of different metals are being made by welding a thin sheet of one metal to a more substantial supporting sheet of the other. For example, a thin sheet of stainless steel has been welded to a sheet of iron or 15 ordinary steel and the composite sheet has been rolled to attempt to eliminate irregularities produced by the welding and to attempt to unite the two sheets throughout their extent. Also, metallic surfaces have been sprayed with molten metal 20 by means of the so-called "metal gun." It has also been attempted to melt one metal and pour it on to another, as for example, the surfacing of iron with molten aluminum, but the aluminum coating is quite irregular and rough when made 25 in this manner. Still another attempt at coating has been made through the use of an electroplating process. This is satisfactory for some purposes, but none of the above methods of coating is sufficiently cheap or sufficiently practicable to be of general application, and none of 30 the above methods of coating is even usable for smoothly coating the entire interior surface of a container such as a barrel.

By way of illustrating an extremely difficult 35 application of the present invention, I am going to show particularly its utility in coating the interior of a beer barrel.

In the past beer barrels have generally been 40 made of wood and coated with pitch or composition. More recently such barrels have been made of metal and the pitch or composition coating has been modified in order to render them adhesive to steel. The frequency with which such coatings require replacement has suggested 45 that the interior of the steel barrel be provided with a metallic coating of such a nature as to resist corrosion and produce no deleterious effect upon the contents of the barrel. Aluminum suggests itself as a desirable material because it is 50 cheap, sufficiently flexible to stand the knocks to which the barrel is subject, substantially non-corrosive, and not in any way harmful to beer. It was found, however, that the aluminum could not satisfactorily be deposited on the interior of 55 the completed barrel by any known means. The

largest opening with which the barrel was provided was altogether too small for any electrode which would be sufficiently large to make electroplating feasible. The most nearly acceptable known method involved the introduction of molten aluminum into the barrel and the discharge therefrom of any surplus. It was found, however, that the thickness of the deposit on the metal could not be accurately gauged and the surface of the deposit was invariably rough and tended to make the barrel unsanitary. While useful for many purposes, this method was not as desirable for this specific purpose as that herein disclosed.

By means of the invention hereinafter to be 15 disclosed, aluminum has been used successfully to line the interior of a steel barrel to produce a smooth and sanitary surface therein. Aluminum is chosen as the example because metallurgists regard the coating of aluminum on steel 20 as being one of the most difficult metallurgical problems. The process and apparatus herein- 25 after to be disclosed are successfully usable for coating with aluminum and may also be used for any other metal, as for example, the surfacing of ordinary steel with special steel such as cobalt or stainless steel.

The drawing shows apparatus of two different 30 forms suitable for carrying out the present invention.

Figure 1 is a plan view of apparatus usable for 35 metallically coating the interior of a barrel.

Figure 2 is an enlarged detail view of the 40 fragment of a barrel in section during the coating operation.

Like parts are identified by the same reference 45 characters throughout the several views.

The apparatus shown in Fig. 1 is substantially 50 a duplicate of that illustrated in my companion application No. 740,662 filed August 20, 1934. In effect it is a centrifuge in which the barrel may be mounted for turning it upon its longitudinal and transverse axes, the whirling on at least one axis being accomplished not only at differing speeds, but also in reverse directions.

The shaft 5 provides a potential rotatable support for a yoke 6 having a headstock 7 and a tailstock 8 detachably engageable with the barrel 10. When the supporting shaft 5 is rotated by means of belt 11, the barrel is turned end for end about a transverse axis. When yoke 6 is horizontal the barrel may be turned on its longitudinal axis and accelerated, decelerated or reversed by engaging the chuck 12 with the squared end of its headstock spindle 7.

Mounted upon the base 15 is a slide 16 carrying a motor 17 which drives the chuck 12 through any suitable reversing gear mechanism.

In order to provide the barrel 10 with a metal-  
5 lic lining the procedure is as follows.

The requisite quantity of aluminum or other metal is provided in powdered form. If the coating is to be of aluminum, the aluminum should preferably be chemically pure and free of those 10 substances commonly mingled with commercial flake aluminum to prevent oxidation. Powdered aluminum of the requisite quality is commercially available.

The powdered metal is preferably mixed with 15 a suitable flux. The flux may, however, be independently coated upon the interior of the barrel if desired. The advantage in mixing the flux with the powdered aluminum consists in the fact that an excess of flux may be used as a vehicle 20 for assisting in the coating of the interior of the barrel with the aluminum. For example, the liquid flux and powdered aluminum may be introduced into the barrel in bulk through the bung hole and the barrel rotated on its support to dis- 25 tribute the aluminum over the interior, after which the surplus flux may be dumped out. The powdered metal may also be sprayed on to the surface to be coated, or in some applications of the invention, it may conveniently be brushed 30 on. The manner of its distribution over the surface to be plated is broadly immaterial.

Having coated with flux and with powdered metal the surface to be plated, said surface is preferably (but not necessarily) heated. In 35 coating steel barrels with aluminum it has been found expedient to heat the barrel to a temperature between 600 degrees F. and 1200 degrees F. 1100 degrees is a very satisfactory temperature. With the barrel thus heated, a large quantity of 40 balls of assorted sizes are introduced into the barrel through the bung hole, as best shown in Fig. 2 in which the balls 20 clearly appear. The number of such balls is broadly immaterial. They may be warm or cold. Ordinary highly 45 polished steel ball bearings have been found to be very useful.

When the balls are in the barrel in sufficient quantities (for example) to fill the barrel from one sixth to one third full, the barrel is rotated 50 on one or both of the axes on which it is mounted for rotation in such an apparatus as that shown in Fig. 1. If the balls achieve the speed of the barrel and rotate unitarily therewith, the rate of motion is either changed or the direction of 55 rotation reversed so that the balls are preferably kept in a state of constant rotative movement respecting the barrel in which they are mounted. Due to the change in rate of movement the balls will tend to change their position 60 in the barrel, and since they are of varying sizes they will roll all interior surfaces thereof. During the end over end rotation of the barrel, which

preferably occurs first, the balls will usually not roll about the surface of the barrel but will be tumbled so as to strike all portions of the surface with a considerable impact.

I have found that both the impact and the 5 rolling are effective to drive the powdered coating material (in this case the powdered aluminum) into the pores of the steel wall of the barrel, with the result that a continuous and relatively non-porous metallic lining is produced. 10 Such a lining completely coats the interior of the barrel, closing and covering all crevices or joints therein and providing a smooth, continuous, imperforate, one piece lining.

Either the rolling or the hammering alone 15 may be used and, as above indicated, the heating of the barrel is not essential to the successful operation of the process, although it facilitates and expedites the production of a smooth 20 lining.

Any suitable flux may be used according to the 25 metals to be joined. The flux may either be applied preliminarily to the supporting metal, or it may be mixed with the powdered metal which is to form the coating.

I claim:

1. The process of lining a metal barrel, which consists in the introduction through a small hole in the barrel of a pulverulent metallic lining material, a suitable flux and a plurality of balls, the heating of the barrel and the rotation thereof, whereby to distribute the lining material in the barrel and to roll it into a continuous coating for the interior thereof.

2. The process of coating a non-cylindrical metal barrel having a small aperture, which process includes the preparation of the interior surface of the barrel to receive the coating, the introduction therein of a pulverulent lining material, and a series of balls in sufficient number 40 to reach all portions of the inner surface of the barrel, the application of heat, and the rotation of the barrel, whereby to distribute the lining material and to roll it into intimately bonded relation to the entire inner surface of the barrel. 45

3. The process of coating the interior of an elongated metallic article which is not perfectly cylindrical on its inner surface, which process includes the preparation of the inner surface of said article to receive a bonded coating, the introduction into the article of a pulverulent metallic lining material, and a number of balls of differing sizes in sufficient quantities to reach all portions of the surface of the article during the rotation thereof, the application of heat, and the 50 rotation of the article, whereby to displace said balls therein and thereby to distribute the lining material and to roll it into intimately bonded relation with the entire inner surface of the article. 55

FREDRICK GETTELMAN.